



US011718952B2

(12) **United States Patent**  
Lim et al.

(10) **Patent No.:** US 11,718,952 B2  
(45) **Date of Patent:** Aug. 8, 2023

(54) **METHOD OF CHEMICAL TREATMENT ON NONWOVENS**

(71) Applicant: **Tintoria Piana, US Inc.**, Cartersville, GA (US)

(72) Inventors: **Sang-hoon Lim**, Kennesaw, GA (US); **Andrea Piana**, Atlanta, GA (US)

(73) Assignee: **Tintoria Piana, US Inc.**, Cartersville, GA (US)

(\*) Notice: Subject to any disclaimer, the term of this patent is extended or adjusted under 35 U.S.C. 154(b) by 451 days.

(21) Appl. No.: **16/880,002**

(22) Filed: **May 21, 2020**

(65) **Prior Publication Data**

US 2020/0378057 A1 Dec. 3, 2020

**Related U.S. Application Data**

(60) Provisional application No. 62/965,240, filed on Jan. 24, 2020, provisional application No. 62/946,484, (Continued)

(51) **Int. Cl.**

**D06M 10/04** (2006.01)  
**D06M 23/16** (2006.01)

(Continued)

(52) **U.S. Cl.**

CPC ..... **D06M 10/04** (2013.01); **A47C 27/002** (2013.01); **D06B 5/08** (2013.01); **D06B 11/0059** (2013.01);

(Continued)

(58) **Field of Classification Search**

None

See application file for complete search history.

(56) **References Cited**

**U.S. PATENT DOCUMENTS**

2002/0193028 A1 \* 12/2002 Zuckerman ..... D06N 3/0061  
442/182

2008/0120761 A1 5/2008 Yang et al.  
(Continued)

**FOREIGN PATENT DOCUMENTS**

CN 201012560 Y \* 1/2008  
EP 594983 A1 \* 5/1994 ..... B05B 3/02  
(Continued)

**OTHER PUBLICATIONS**

English machine translation of Liang (CN 201012560 Y) accessed online from Espacenet; PDF pp. 1-11. (Year: 2010).\*

(Continued)

*Primary Examiner* — Katie L. Hammer

(74) *Attorney, Agent, or Firm* — WC&F IP

(57) **ABSTRACT**

Nonwovens having low-density and resilience have a chemical formulation applied on one surface (e.g., a top surface) by any of various application methods. Then, the chemical formulation is forced to move toward the opposite surface of the nonwoven (e.g., move downward through the nonwoven from top to bottom). The chemical-treated nonwoven is dried to fix the chemical on the nonwovens. Movement through the nonwoven is performed in a controlled fashion so that after drying the distribution of a chemical formulation throughout the nonwoven (e.g., from the top surface to the bottom surface of a nonwoven) is controlled.

**10 Claims, 2 Drawing Sheets**



|                      | <b>Related U.S. Application Data</b>                                                                                                                                                                                  | (56) | <b>References Cited</b>                                                                                              |
|----------------------|-----------------------------------------------------------------------------------------------------------------------------------------------------------------------------------------------------------------------|------|----------------------------------------------------------------------------------------------------------------------|
|                      | filed on Dec. 11, 2019, provisional application No. 62/946,173, filed on Dec. 10, 2019, provisional application No. 62/882,279, filed on Aug. 2, 2019, provisional application No. 62/854,547, filed on May 30, 2019. |      | U.S. PATENT DOCUMENTS                                                                                                |
| (51) <b>Int. Cl.</b> |                                                                                                                                                                                                                       |      |                                                                                                                      |
|                      | <i>D06M 23/12</i> (2006.01)                                                                                                                                                                                           |      | 2008/0121461 A1 5/2008 Gross et al.                                                                                  |
|                      | <i>A47C 27/00</i> (2006.01)                                                                                                                                                                                           |      | 2009/0162621 A1 * 6/2009 Craamer .....                                                                               |
|                      | <i>D06M 23/02</i> (2006.01)                                                                                                                                                                                           |      | ..... D06M 16/00<br>427/75                                                                                           |
|                      | <i>D06P 5/30</i> (2006.01)                                                                                                                                                                                            |      | 2009/0288259 A1 * 11/2009 Lean .....                                                                                 |
|                      | <i>D06B 5/08</i> (2006.01)                                                                                                                                                                                            |      | B29C 70/64<br>264/45.4                                                                                               |
|                      | <i>D06B 11/00</i> (2006.01)                                                                                                                                                                                           |      | 2017/0020299 A1 * 1/2017 Valenta .....                                                                               |
|                      | <i>D06B 19/00</i> (2006.01)                                                                                                                                                                                           |      | A47C 21/046                                                                                                          |
|                      | <i>D06M 101/32</i> (2006.01)                                                                                                                                                                                          |      | 2018/0230647 A1 8/2018 Petton et al.                                                                                 |
| (52) <b>U.S. Cl.</b> |                                                                                                                                                                                                                       |      | FOREIGN PATENT DOCUMENTS                                                                                             |
|                      | CPC ..... <i>D06B 19/0094</i> (2013.01); <i>D06M 23/02</i> (2013.01); <i>D06M 23/12</i> (2013.01); <i>D06M 23/16</i> (2013.01); <i>D06P 5/30</i> (2013.01); <i>D06M 2101/32</i> (2013.01)                             |      | EP 678614 A2 * 10/1995 .....                                                                                         |
|                      |                                                                                                                                                                                                                       |      | D06B 1/06                                                                                                            |
|                      |                                                                                                                                                                                                                       |      | EP 1350452 A1 * 10/2003 .....                                                                                        |
|                      |                                                                                                                                                                                                                       |      | A47G 9/0215                                                                                                          |
|                      |                                                                                                                                                                                                                       |      | OTHER PUBLICATIONS                                                                                                   |
|                      |                                                                                                                                                                                                                       |      | English machine translation of Wehrli (EP 1 350 452 A1) accessed online from Espacenet; PDF pp. 1-16. (Year: 2003).* |
|                      |                                                                                                                                                                                                                       |      | * cited by examiner                                                                                                  |

Chemical application (deposition)

Chemical distribution

Drying

FIG. 1



FIG. 2



FIG. 3

## METHOD OF CHEMICAL TREATMENT ON NONWOVENS

### CROSS-REFERENCE TO RELATED APPLICATIONS

This application claims priority to U.S. Provisional Application 62/854,547 filed May 30, 2019, U.S. Provisional Application 62/882,279 filed Aug. 2, 2019, U.S. Provisional Application 62/946,173 filed Dec. 10, 2019, U.S. Provisional Application 62/946,484 filed Dec. 11, 2019, and U.S. Provisional Application 62/965,240 filed Jan. 24, 2020, and the complete contents of each of these applications is herein incorporated by reference.

### FIELD OF THE INVENTION

Aspects of the invention are generally related to a method to apply chemical formulations on nonwovens having resilience and low density. It provides a method to control the distribution of the chemical formulations applied on one surface of the nonwovens toward the opposite surface of the nonwovens.

### BACKGROUND

Chemical treatment on woven or knitted fabrics is normally done by a pad-dry-cure method. In this method, the fabric is passed through a chemical bath for complete soaking. Then, an excess amount of chemical is removed from the woven or knitted fabric by passing it through a pair of squeezing rollers. Finally, the woven or knitted fabric is dried and cured to fix the chemicals on the fabric. This method might be used for high-density nonwovens, whose shapes are not much affected by the soaking and squeezing. However, the nonwovens with low density and bulkiness cannot be treated with chemicals by a pad-dry-cure method since the nonwovens will lose their shapes by the soaking and squeezing. Also, the physical strength of the nonwovens is generally not strong enough to sustain the process and they will be damaged after the process. Thus, there is a need for a method that applies chemical formulations on the nonwovens with minimal damage to them.

### SUMMARY

In an embodiment of the invention, a chemical formulation is applied on one surface of a nonwoven having resilience and low density by various application methods, and the chemical formulation is forced to move through the body of the nonwoven toward the opposite surface of the nonwoven. The chemical-treated nonwoven is dried to fix the chemical on the nonwoven. The distribution of a chemical formulation from one surface to the opposite surface of a nonwoven may also be controlled in various embodiments of the invention.

### DESCRIPTION OF THE DRAWINGS

FIG. 1. is a general scheme of the inventive process; FIG. 2. is an order set of side views of nonwovens at each step of the process; and

FIG. 3. is an illustration of a table-top digital printer which may be used in the practice of the invention.

### DETAILED DESCRIPTION

Aspects of the invention are generally related to a chemical treatment method for use on nonwovens having low-

density and resilience. In this application, the low-density nonwovens are defined as the nonwovens that have a density ranging from 0.15 g/cm<sup>3</sup> (gram/cubic centimeter) to 0.001 g/cm<sup>3</sup> (or below). Nonwovens with resilience are defined as nonwovens that have a thickness loss of not more than 80% after the entire chemical treatment process comprising chemical application, chemical distribution, and drying steps. Nonwovens of low-density and resilience are available from a number of commercial sources including Piana 10 Nonwovens LLC (Cartersville, Ga.).

A nonwoven is a manufactured sheet, web, or batt of natural and/or man-made fibers or filaments that are bonded to each other by any of several means. Manufacturing of nonwoven products is well described in "Nonwoven Textile Fabrics" in Kirk-Othmer Encyclopedia of Chemical Technology, 3rd Ed., Vol. 16, July 1984, John Wiley & Sons, p. 72-124 and in "Nonwoven Textiles", November 1988, Carolina Academic Press. Web bonding methods include mechanical bonding (e.g., needle punching, stitch, and 15 hydro-entanglement), chemical bonding using binder chemicals (e.g., saturation, spraying, screen printing, and foam), and thermal bonding using binder fibers with low-melting points. Two common thermal bonding methods are air heating and calendering. In air heating, hot air fuses 20 low-melt binder fibers within and on the surface of the web to make high-loft nonwoven. In the calendering process, the web is passed and compressed between heated cylinders to 25 produce a low-loft nonwoven.

The vertically lapped nonwoven material can be produced 30 by commercially available machines, such as V-Lap vertical lapping systems sold by V-Lap Pty Ltd. and by Struto International, Inc. In the V-Lap system, staple fiber blend including binder fibers are opened, blended, and carded. The carded fiber web is pleated and the fibers are bonded 35 mechanically (needling) and thermally to produce vertically lapped nonwovens. In the Struto system, the carded fiber web containing binder fiber is fed into the Struto lapping device. The vertical lapper then folds the web into a uniform structure. The folds are compressed together into a continuous 40 structure, which is held in vertical position as it passes the heated thermal bonding oven. Due to its vertical fiber arrangement, the vertically lapped nonwovens provide better resilience and shape recovery to compression compared to cross lapped nonwovens.

45 Any type of nonwoven can be used for this application as long as it is within the specification of the resilience and density described in this application. (thickness loss not more than 80% after the entire chemical treatment process and a density of 0.15 g/cm<sup>3</sup> or below). The preferred 50 nonwovens for this application are thermal-bonded vertically lapped nonwovens and thermal-bonded cross lapped nonwovens.

When nonwovens are made with elastomeric binder fibers and high resilience fibers, it provides a better resilience to 55 the nonwovens. As examples of the elastomeric polyester binder fibers, these include but are not limited to ELK®, E-PLEX®, and EMF type high elastic LMF that are commercially available from Teijin Limited, Toray Chemical Korea Inc., and Huvis Corporation, respectively. The elastomeric polyester binder fiber provides an elastic property to the nonwoven and provides bonding between fibers after the thermal bonding process. To provide bulkiness and resilience to the nonwoven, hollow conjugate polyester fiber can be used together with binder fibers, such as the elastomeric 60 binder polyester fiber, conventional binder fibers, or any combination of these. In addition to these fibers, other fibers 65 can be used to give other required functions. Other fibers

include but not limited to man-made (e.g., rayon, lyocell, Nylon, Kevlar, etc.) and/or natural fibers (e.g., cotton, jute, silk, wool, linen, cashmere, etc.). Exemplary types of polyesters include but are not limited to PET (polyethylene terephthalate), PTT (polytrimethylene terephthalate), and PBT (polybutylene terephthalate). The most commonly used polyester is PET.

Examples of fiber blends for the cross lapped and vertically lapped nonwovens having low-density and resilience that could be used in the practice of this invention include but are not limited to the following:

Elastomeric polyester binder fiber (6 denier×64 mm):

High shrink polyester fiber (1.4 denier×51 mm): Low-melt polyester binder fiber (4 denier×51 mm): Regular polyester fiber (6 denier×51 mm)=25:20:10:45

Hollow conjugate polyester fiber (3 denier×51 mm):

Elastomeric polyester binder fiber (6 denier×64 mm)=60:40

Hollow conjugate polyester fiber (15 denier×51 mm):

Elastomeric polyester binder fiber (6 denier×51 mm)=60:40

Hollow conjugate polyester fiber (15 denier×51 mm):

Low-melt polyester binder fiber (4 denier×51 mm)=70:30

Hollow conjugate polyester fiber (3 denier×51 mm): High shrink polyester fiber (1.4 denier×51 mm): Elastomeric

polyester binder fiber (6 denier×64 mm): Low-melt polyester binder fiber (4 denier×51 mm)=40:20:30:10

Hollow conjugate polyester fiber (3 denier×51 mm): High

shrink polyester fiber (1.4 denier×51 mm): Elastomeric polyester binder fiber (6 denier×64 mm)=50:10:40

Hollow conjugate polyester fiber (3 denier×51 mm):

Hollow conjugate polyester fiber (15 denier×51 mm):

Elastomeric polyester binder fiber (6 denier×64 mm):

Low-melt polyester binder fiber (4 denier×51 mm)=50:25:15:10

FIG. 1 shows the general scheme of the process, which comprises chemical application (deposition), chemical distribution, and drying. While FIG. 1 illustrates a three step process, other process steps may be performed before, after, and in between the three steps. The chief requirement is that the steps of deposition, distribution and drying are performed, and that the distribution step follows the deposition step, and that the drying step follows the distribution step. FIG. 2 illustrates side views of nonwovens (vertically lapped or not vertically lapped) at each step of the process.

The first step of the process is a chemical application step. A chemical formulation (for example, in a liquid form) is applied on one surface of the nonwoven having low-density and resilience. Generally speaking, it will be applied on the top surface in any desired pattern, and using any of a variety of application techniques including but not limited to inkjet technology, valve jet technology, spraying, foam application, digital printing, roller coating, doctor blade coating, and screen/rotary printing. Using these chemical deposition methods, the chemical formulation will reside mostly on the top surface of the nonwoven.

For the chemical formulations for the invention, any chemicals can be used. In some embodiments of this invention, chemicals used for this application provide functionality to the nonwovens. Exemplary chemicals include but not limited to water/oil repellents, antimicrobials, flame retardants, microencapsulated scents, microencapsulated cosmetics, microencapsulated essential oils, microencapsulated PCM (Phase Change Material), probiotics, odor control agents, photocatalytic agents, UV absorbers, anti-allergens, probiotics, hydrophilic agents, hand modifying agents,

antistatic agents, insect repellents, and ceramics that emit far infrared and/or negative ions. The chemical formulations may include two or more different agents and/or two or more of the same class of agents (e.g., two different UV absorbers and one antistatic agent). The chemical formulations are preferred to be in liquid form such as aqueous or oil based solutions or dispersions in liquid form. In some applications, these chemicals can be combined to provide multi-functions on the treated nonwovens. In some applications, colors can be added to the formulation. An example chemical formulation that can be applied to a nonwoven comprises micro-encapsulated PCM, binder, wetting agent, and water.

Although any chemical application methods can be used for the invention, one of the preferred chemical application methods involves the use of a non-contact digital chemical deposition technology (e.g., digital printers, etc.). The technology allows deposition of chemical formulations on the nonwovens without physical contact between the chemical dispensing parts (e.g., nozzles or outlets) and nonwovens. Since it eliminates the physical stress that results from soaking and squeezing which are part of a pad-dry-cure process, the damage on the low-density nonwoven during chemical application is eliminated or minimized. An example of a non-contact digital chemical deposition technology that can be used for this invention includes but is not limited to CHROMOJET digital printing system from Zimmer based in Austria. A small laboratory sample can be prepared by a table-top digital printer as shown on FIG. 3.

In some applications, different chemicals can be combined to provide multi-functions on the nonwoven using a digital printing system. FIG. 3 shows by example, using multiple printing modules 30 with different chemicals in the modules (for example, a module A could contain antimicrobial finish and module B could contain microencapsulated PCM). In addition, different chemical formulation tanks 32 could be connected to different printing modules 30. This set up allows the different chemicals to be applied on a nonwoven at the same time. In some applications, colors can be added to the chemical formulation, or themselves be provided in a separate module for simultaneous application to the nonwoven. In applications where functionality is the primary concern, the digital printing system may be used to cover the majority of or the entire nonwoven with the functional chemical (i.e. the chemical is printed across the entire surface of nonwoven or a majority of the surface). However, in some applications it may be advantageous to print functional chemicals in a pattern which covers less than the entire nonwoven (e.g., in some applications, micro-encapsulate scents might be printed only in certain parts of the nonwoven, etc.). An example chemical formulation that can be digitally printed onto a low-density nonwoven with resilience comprises water repellent, binder, water, and printing auxiliaries, such as thickener and wetting agent.

One of the benefits of using a digital printing system for chemical application is to control the depth of chemical deposit on the nonwoven that is treated to a certain extent. The depth of chemical penetration and the amount of chemical applied on the nonwoven can be controlled by many variables, such as viscosity of the formula, the pressure applied to the formulation that is ejected through the nozzle, printing speed, printing resolution, pressing after printing, density of nonwovens, and so on.

The nonwoven for the treatment can be a single layer nonwoven or multilayer nonwovens. The multilayer nonwovens may be comprised of two or more layers of nonwovens, whose layers may be bonded together.

At some point after application of the chemical formulation to the nonwoven having low-density and resilience, chemical distribution is performed. The chemical distribution step is a physical step which causes the layer or deposited islands of the chemical formulation on a surface of a nonwoven to be physically distributed throughout the thickness of the nonwoven. In this step, the chemical formulation mainly resides on the surface to which it is applied (e.g., on the top surface) of the nonwoven although some portions of the chemical formulation may reside under the surface depending on the density of the nonwoven. During chemical distribution, the chemical formulation is forced to move through the nonwoven to the opposing surface (e.g. down toward the center or bottom of the nonwoven). The objective of chemical distribution is that after it is performed, the chemical formulation will no longer primarily reside on one surface (e.g., the top surface) of the nonwoven. The preferred chemical distribution method is pressing the nonwoven using at least one pair of press rollers. However, any type of pressing method can be utilized, and it can include but is not limited to using at least one pressing plate that presses down on the top surface of the nonwoven, or using at least one pressing top roller with a bottom moving conveyer carrying the nonwoven. In some embodiments, any non-pressing method can be used to distribute the chemical formulation from one surface of the nonwoven toward the opposite surface of the nonwoven, and this includes but is not limited to vacuum suction from the opposite surface of the nonwoven.

Not all compressive forces will be bad for nonwovens prepared according to this invention. For example, a cross lapped or vertically lapped nonwoven with resilience and good shape stability can be passed through a pair of press rollers after chemical application without noticeable structural deformation. By passing through the pair of press rollers, the chemicals applied on the nonwoven can be penetrated further down from the application surface of the nonwoven. The depth of the penetration is controlled by the gap and pressure between the rollers. The gap can be 0 mm or above depending on the depth of chemical penetration required. The main function of the press rollers is to make the applied chemical on the surface of the nonwoven move down through the nonwoven material, not to squeeze excess chemical from the nonwoven. By controlling the pressure or the gap, it would be, for example, to have the chemical move only from the surface on which it is applied to a middle portion of the nonwoven or to the opposite side of the nonwoven (e.g., 25% through, 50% through, 75% through, 100% through, etc.). For example, in some applications where the nonwoven is a multiple layered material, the chemical distribution step may be controllably performed to distribute the chemicals only in the top one or two layers and not have it distributed to the bottom one or two layers.

After distribution of chemical in the desired fashion, the nonwoven is dried primarily to fix chemicals on the nonwoven. But, in some embodiments, drying is also used to remove water/solvent from the chemical formulation. If needed, the nonwoven, after being dried, goes to a curing step.

FIG. 2 illustrates a variation on the methodology of FIG. 1 and is particularly suited to low-density nonwovens (vertically lapped or not vertically lapped) having resilience against some pressure applied by press rollers. In FIG. 2, the first step is to apply (deposit) a layer of a chemical formulation in liquid form in the same manner as shown in FIG. 1. Then, the nonwoven is passed through one or more pairs of press rollers. As shown in the last two panels of FIG. 2,

the pressing action helps drive the chemical formulation down into the interior of the nonwoven, i.e., the chemical formulation will no longer primarily reside on the surface of the nonwoven. As illustrated in the second to last and last panel, more pressure can lead to a full penetration of the chemical formulation from the application side through the thickness to the opposing side of the nonwoven while less pressure application can lead to, for example, a half penetration. Depending on the final use of the product and its application, the chemical penetration depth can be controlled by controlling the amount of pressure and/or the gap of the pair of press rollers.

In one embodiment, a colorant is included in the chemical formulation and can be used as a gauge to demonstrate penetration of the chemical formulation into and/or through the thickness of the nonwoven. As discussed above, the chemical formulation may include water/oil repellents, antimicrobials, flame retardants, microencapsulated scents, microencapsulated cosmetics, microencapsulated essential oils, microencapsulated PCM (Phase Change Material), probiotics, odor control agents, photocatalytic agents, UV absorbers, anti-allergens, probiotics, hydrophilic agents, hand modifying agents, antistatic agents, insect repellents, and ceramics that emit far infrared and/or negative ions. Specifically, with referenced to FIG. 2, it can be seen that a layer of the chemical formulation with a colorant 20 (which can be continuous as shown, or which can be discontinuous) on the surface of the nonwoven 22 is subjected to physical distribution throughout the nonwoven by press rollers 24. Depending on such factors as the amount of pressure applied to the rollers 24, the weight of the rollers 24, the gap between the rollers 24, and the fibers in the nonwoven 22 and its construction, the chemical formulation can be distributed throughout the thickness of the nonwoven 22, or be only partially distributed. With colorant, the manufacturer may be able to more easily control how far chemicals in the chemical formulation are distributed into the nonwoven after a surface application using for example, an inkjet technology such as an inkjet printer. Of course, the process could be performed without a colorant depending on the needs of the manufacturer. The chemical-treated nonwoven goes to a drier to dry water/solvent from the formulation and/or to fix chemicals on the nonwoven.

The chemical-treated nonwovens in the invention can be used for a variety of applications such as, but not limited to consumer products, bedding, furniture, automotive, and airplane. For example, a nonwoven layer treated with microencapsulated PCM can be placed under a ticking fabric of mattresses to provide comfort to the user or used for mattress toppers.

As it will be apparent to those of skill in the art upon reading this disclosure, each of the individual embodiments described and illustrated herein has discrete components and features which may be readily separated from or combined with the features of any of the other several embodiments without departing from the scope or spirit of the present invention. Any recited method can be carried out in the order of events recited or in any other order which is logically possible.

The invention is further described by the following non-limiting examples which further illustrate the invention, and are not intended, nor should they be interpreted to, limit the scope of the invention.

#### EXAMPLE 1

A chemical formulation comprising microencapsulated scent (camomile), a binder, a thickener, a wetting agent, and

water was applied on a cross lapped nonwoven made with 70% hollow conjugate polyester fiber (3 denier, 51 mm) and 30% Teijin ELK fiber (6 denier, 64 mm) using a table-top digital printing machine (table-top CHROMOJET by Zimmer Austria). The basis weight of the nonwoven was 225 gsm (grams/m<sup>2</sup>). The amount of the chemical formulation applied on the nonwoven was 70 gsm. The nonwoven was dried in an oven at 120° C. until the formulation was completely dried. The dried chemical formulation resided mostly on the top surface of the nonwoven. The microencapsulated capsules release a scent when pressure or friction is applied on the nonwoven.

## EXAMPLE 2

A chemical formulation comprising microencapsulated PCM, a binder, a thickener, a wetting agent, a blue reactive dye, and water was applied on a vertically lapped nonwoven made with 70% hollow conjugate polyester fiber (3 denier, 51 mm) and 30% Teijin ELK fiber (6 denier, 64 mm) using a table-top digital printing machine (table-top CHROMOJET by Zimmer Austria). The basis weight of the nonwoven was 600 gsm (grams/m<sup>2</sup>). The amount of the chemical formulation applied on the nonwoven was 900 gsm. The chemical-applied nonwoven was passed through a pair of press rollers to force the chemical formulation on the surface of the nonwoven toward the bottom of the nonwoven. The gap between rollers was 0 mm and the pressure applied on the rollers was 0.4 MPa. Then, it was dried in an oven at 120° C. until the formulation was completely dried. Then it was cured 160° C. for 3 min. The dried chemical formulation was well distributed through the whole entire nonwoven as indicated by blue color. This final nonwoven has a cooling function due to the microencapsulated PCM and one of example use of this is for mattress.

While the present invention has been described in terms of preferred embodiments, those skilled in the art will recognize that the invention can be practiced with considerable modification within the spirit and scope of the appended claims.

It is noted that, as used herein and in the appended claims, the singular forms "a", "an", and "the" include plural referents unless the context clearly dictates otherwise. Having thus described the invention in rather full detail, it will be understood that such detail need not be strictly adhered to, but that additional changes and modifications may suggest themselves to one skilled in the art, all falling within the scope of the invention as defined by the subjoined claims.

The invention claimed is:

1. A chemical treatment method for a nonwoven, comprising:  
 applying a chemical formulation to one surface of a nonwoven comprised of a manufactured sheet, web, or batt of natural and/or man-made fibers or filaments that are bonded to each other having low-density ranging from 0.15 g/cm<sup>3</sup> to 0.001 g/cm<sup>3</sup>; then  
 distributing the chemical formulation through a thickness of the nonwoven by a physical process; and then  
 drying the chemical formulation distributed within the nonwoven after the distributing step,  
 wherein the nonwoven has a resilience of having a thickness loss of not more than 80% after performing the steps of applying, distributing and drying, wherein the chemical formulation includes phase change materials (PCMs).

2. The chemical treatment method of claim 1, wherein said applying step is performed using an application device selected from the group consisting of non-contact digital chemical deposition technology, valve jet technology, spraying, foam application, digital printing, roller coating, doctor blade coating, and screen/rotary printing.

3. The chemical treatment method of claim 1 wherein said chemical formulation further includes one or more of water/oil repellents, antimicrobials, flame retardants, microencapsulated scents, microencapsulated cosmetics, microencapsulated essential oils, probiotics, odor control agents, photocatalytic agents, UV absorbers, anti-allergens, probiotics, hydrophilic agents, hand modifying agents, antistatic agents, insect repellents, and ceramics that emit far infrared and/or negative ions.

15 4. The chemical treatment method of claim 3 wherein said chemical formulation further includes at least one colorant.

5 5. The chemical treatment method of claim 1 wherein said distributing step is performed using a pressing plate, a pair of press rollers, or vacuum suction.

10 6. A chemical treatment method, comprising:  
 applying using a non-contact digital chemical deposition technology a chemical formulation on a first surface of a nonwoven comprised of a manufactured sheet, web, or batt of natural and/or man-made fibers or filaments that are bonded to each other which has a low-density ranging from 0.15 g/cm<sup>3</sup> to 0.001 g/cm<sup>3</sup>, wherein said nonwoven has second surface opposing said first surface and separated by a thickness; then

15 25 30 35 physical distributing the chemical formulation from the first surface through the thickness toward the second surface by either applying a pressing force on the first surface or applying a suction force on the second surface; and then

drying the chemical formulation on the nonwoven, wherein the chemical formulation includes phase change materials (PCMs).

7. The chemical treatment method of claim 6, wherein the nonwoven is resilient.

40 8. The chemical treatment method of claim 6, wherein the non-contact digital chemical deposition technology is a digital printer.

9. The chemical treatment method of claim 6, wherein the chemical formulation further includes one or more of water/oil repellents, antimicrobials, flame retardants, microencapsulated scents, microencapsulated cosmetics, microencapsulated essential oils, probiotics, odor control agents, photocatalytic agents, UV absorbers, anti-allergens, probiotics, hydrophilic agents, hand modifying agents, antistatic agents, insect repellents, and ceramics that emit far infrared and/or negative ions.

50 45 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 95